

## UNITED STATES PATENT OFFICE

STERLING H. DIGGS, OF CASPER, WYOMING, ASSIGNOR TO STANDARD OIL COMPANY, OF WHITING, INDIANA, A CORPORATION OF INDIANA

## FUEL OIL

No Drawing.

Application filed January 16, 1928. Serial No. 247,264.

This invention relates to the production of fuel oil from acid sludge. In the ordinary way of working up acid sludge, as much acid as possible is recovered. This may be done by diluting the sludge with naphtha bottoms or similar oils and water and heating while subjecting to agitation. Thereafter, the mixture is allowed to settle, whereupon it divides into a lower aqueous layer consisting mainly of dilute sulfuric acid and a supernatant layer of oily and tarry substances.

In converting the acid sludge tar into fuel oil, for example, railroad fuel oil, it has heretofore been the practice to reduce the tar with steam so as to recover valuable naphtha bottoms therefrom and to cut-back the residue to the desired viscosity with a cheap diluent to give a fuel of satisfactory viscosity. Suitable cut-backs are high sulfur gas oil, and reduced high pressure tar.

Fuel oil produced in this manner is per se satisfactory for combustion in locomotive and other burners. It has, however, an outstanding disadvantage in that on mixing with certain standard fuels of the same general type, an excessive quantity of bottom settling is produced. Thus, when such a fuel oil is mixed with a railroad fuel derived from a residue containing large quantities of waxy and asphaltic materials, the amount of bottom settling from the mixture may amount to several times the amount which would be anticipated from the bottom settling of each of the constituents. An example of such a fuel oil is that produced from reduced pressure tar from Burton or Burton-Clark cracking stills. This disadvantage has heretofore prevented the utilization of sludge tar for the production of commercial fuel because of the certainty that in actual practice, the two kinds of fuel would become mixed in supply tanks and storage tanks and the burners and feed-pipes would become choked.

It has now been discovered that this difficulty can be completely avoided by conducting the reduction of the sludge tar under such conditions that the temperature exceeds 500° and preferably attains temperatures between 550 and 600° F. The result of this high tem-

perature seems to be the breaking up of oxygen and sulfur compounds present in the sludge tar, which apparently were responsible for the excessive settling from the mixed fuel oils. Higher temperatures may be employed, if desired, but are not necessary for the accomplishment of the desired result.

The invention will be readily understood from the following description of a preferred example.

Sludge tar derived on separation from the acid layer and containing about 50% of naphtha bottoms is heated to a high temperature and the naphtha bottoms recovered and condensed. The heating may be effected in a pipe still or in a shell still. When the latter is employed, it is preferred to inject a small amount of steam so as to give enough agitation to prevent the settling of insoluble matter on the bottom thereof. During this heating, the temperature is caused to rise above 500° F. and preferably between 550 and 600° F. The viscosity of the residue is relatively unimportant and it varies considerably, for example, from 300 to 1000 furul at 122° F. The steam-reduced tar is now cut back by addition of an oil of less viscosity until a fuel oil meeting the specifications results. For railroad fuels, the viscosity must usually not exceed 60 furul at 122° F. and it is preferred to reduce the viscosity to below 40, for example, 35 or lower. The amount of diluent is relatively small, for example, a mixture of 40% of oil having a viscosity of 10 and 60% of an oil having a viscosity of 600 will have a viscosity of about 35.

In actual practice, it is desired to blend the reduced steam tar or bottoms with other fuel oils, for example, a fuel oil having a viscosity of about 25 furul at 122° F. derived from the distillation of pressure tar from cracking operations of the Burton or Burton-Clark type.

I claim:

1. The method of producing fuel oil from acid sludge which consists in adding thereto a hydrocarbon oil of low viscosity, and water, heating with agitation, separating the hydrocarbon constituents from the

aqueous acid solution, heating said hydrocarbon mixture to expel the added hydrocarbons of low viscosity, raising the temperature to between 500 and 600° F., and cutting-back the residue with fuel oil constituents of relatively low viscosity to give a blended fuel of desired viscosity.

- 5 2. The method of producing fuel oil from acid sludge which consists in adding there-to to a hydrocarbon oil of low viscosity and water, heating with agitation, separating the hydrocarbon constituents from the aqueous acid solution, heating said hydrocarbon mixture to expel the added hydrocarbons of low
- 10 15 viscosity, raising the temperature to between 500 and 600° F., and mixing the residue with a residual fuel from a cracking operation of the Burton type, to give a blended fuel of desired viscosity.
- 15 20 3. The method of making fuel oil which consists in separating a hydrocarbon layer containing oxygen and sulfur compounds from acid sludge, heating said layer of hydrocarbon compounds to a temperature be-
- 25 30 tween about 500 and about 600° F., thereby driving off the more volatile constituents, and cutting-back the residue to a desired viscosity with fuel oil constituents of relatively low viscosity.
- 30 35 4. The process of converting acid sludge tar containing insolubilizing oxygen and sulfur compounds into an oil which may be mixed with fuel oils without mutual pre-
- 35 40 cipitation of objectionable sludge com-pounds comprising heating said acid tar above a temperature of about 500° F. and not substantially above 600° whereby said oxygen and sulfur compounds are decom-posed and then reducing the viscosity of the resulting oil by adding a small proportion of a low viscosity fuel oil.

STERLING H. DIGGS.

45

50

55

60

65